# EUROPEAN PATENT SPECIFICATION

(11) **EP 1 440 751 B1**
(45) Date of publication and mention of the grant of the patent: **14.03.2007**
(21) Application number: 04000274.3
(22) Date of filing: 08.01.2004
(51) Int. Cl.: B22F 1/00, C22C 33/02

(54) **Production method of a sintered body**
Herstellungsverfahren eines Sinterkörpers
Procédé de production d'un corps fritté

(30) Priority: 17.01.2003 JP 2003009483
(43) Date of publication of application: 28.07.2004
(73) Proprietor: NISSAN MOTOR COMPANY LIMITED, Yokohama-shi Kanagawa 221-0023 (JP); JFE Steel Corporation, Tokyo, 100-0011 (JP)
(72) Inventor: Unami, Shigeru, JFE Steel Corporation, Chiyoda-ku Tokyo 100-0011 (JP); Uenosono, Satoshi, JFE Steel Corporation, Chiyoda-ku Tokyo 100-0011 (JP); Mabuchi, Yutaka, Yokohama-shi Kanagawa 231-0834 (JP); Fujiki, Akira, Yokohama-shi Kanagawa 236-0023 (JP); Maekawa, Yukihiro, Yokohama-shi Kanagawa 233-0002 (JP); Murata, Takashi, Yokohama-shi Kanagawa 233-0015 (JP)
(74) Representative: Weber, Joachim

(56) References cited:
- US-A- 2 637 671
- US-A- 4 588 441
- US-A- 5 540 883
- US-B1- 6 332 904
- PATENT ABSTRACTS OF JAPAN vol. 2003, no. 08, 6 August 2003 (2003-08-06) -& JP 2003 096533 A (KAWASAKI STEEL CORP; NISSAN MOTOR CO LTD), 3 April 2003 (2003-04-03)

## Description

### BACKGROUND OF THE INVENTION

The present invention relates to a powder metallurgy technique for producing a sintered metal body having excellent fatigue strength and abrasion resistance to be suitable for use in a sprocket of a silent chain at low cost.

Various techniques have been proposed to increase green density and sintered density for improvement in sinter strength. In one proposed technique, a sintered body is produced by compacting a metal powder material repeatedly and then sintering the compacted powder material repeatedly. In another technique (disclosed in Japanese Laid-Open Patent Publication No. 2001-295915), a sintered body is produced by warm-compacting a metal powder material and sintering the compacted powder material at elevated temperatures.

### SUMMARY OF THE INVENTION

However, the former technique results in relatively high production cost. The latter technique may allow cost reduction, but has a limitation of improvement in sinter strength. For further improvement in sinter strength (notably fatigue strength and abrasion resistance), it is necessary to reduce the size of pores in the sintered body, strengthen particle-to-particle bonding of the sintered body and thereby prevent the occurrence and development of cracking in the sintered body. The proposed techniques are not always effective in pore size reduction and particle-to-particle bond strengthening and are no more than the modifications of the compacting and sintering processes.

JP 2003-096533 corresponding to an application which has been filed prior to the priority date of the present case but published after the priority date discloses a sintered body comprising an iron-based powder mixture within iron-based powder having a maximum particle size of primary particles equal or smaller than 75 µm and graphite powder in an amount of 0,1 to 1,0 % by mass.

US 2 637 671 discloses a powder mixture comprising metal powders and graphite in an amount of 0,4 to 1,5 wt %. The powders may be finer than 200 mesh. Furthermore, lubricant in an amount of 0,5 to 1 % may be added.

US 4 588 441 also discloses a mixture for powder metallurgy. The mixture comprises iron powders with a diameter of less than 30 micron. Lubricant and graphite may also be included.

US-B-6332904 discloses a sintered body with good fatigue strength and abrasion resistance, e.g. for use in a sprocket. However, the maximum particle size differs from the inventive particle size being 100 µm or smaller.

US-A-5540883 discloses a method for producing a bearing from a powder metal material, which is mainly composed of iron powder and blended with carbon, ferro alloys and lubricant. The bearing is then produced by forming the powder metal material into a blank and sintering the thus-obtained blank at 1250 to 1350 °C in a reducing atmosphere. The ferro alloy has a particle size of up to 25 microns before sintering. The particle size of the elemental iron powder is much larger than the particle size of the ferro alloy. Due to such a large particle size of the elemental iron powder, the sintered metals of the bearing will not have a maximum particle size of 100 µm or smaller.

It is an object of the present invention to provide a sintered body that has sufficiently improved fatigue strength and abrasion resistance.

According to the invention, the object is solved by the features of the main claim. The sub-claims contain further preferred developments of the invention.

The other objects and features of the invention will also become understood from the following description.

### BRIEF DESCRIPTION OF THE DRAWINGS

FIG 1 is a graph showing the abrasion performance of sintered bodies of Examples 1 to 4 illustrating the present invention:

FIG 2 is a graph showing the abrasion performance of sintered bodies of Comparative Examples 1 to 4 according to the earlier technology.

FIG 3 is an optical micrograph of the sintered body of Example 3.

FIG. 4 is an optical micrograph of the sintered body of Comparative Example 3.

### DETAILED DESCRIPTION OF THE INVENTION

The present invention will be described below in detail. In the following description, all percentages (%) are by mass unless otherwise specified.

As a result of extensive researches, the present inventors have found that the use of a fine powder as a raw material allows substantial reduction of the size of pores in a sintered body in addition to increase in the compactness of a green compact. The present inventors have also found that the use of such a fine powder strengthens particle-to-particle bonding of the sintered body, because the fine powder allows promoted diffusion of powder particles during sintering due to a large particle surface. Although the fine powder is generally low in compactibility, the present inventors have found that the compactibility of the fine powder can be improved by the combination of die lubrication and warm compaction. Further, the present inventors have found that the sintering of the compacted fine powder at a high temperature maximizes the particle diffusion, thereby attaining sinter strength higher than ever before. The present invention has been made based on the above findings.

According to the present invention, a sintered body is produced by preparing a metal powder mixture, compacting the metal powder mixture to provide a green compact, and then, sintering the green compact.

The metal powder mixture includes a fine metal powder, a graphite powder and a powder lubricant.

The fine metal powder usable in the metal powder mixture is not particularly restricted and can be selected among various powder metallurgical materials, such as carbon steel powders and alloyed steel powders, depending on the performance required of the sintered body. In the case of the fine metal powder containing an alloy component, the metal powder may be in the form of a completely alloyed steel powder (prepared by the melting and powdering of a desired steel composition), a partially diffusion-alloyed steel powder (prepared by the diffusion joining of alloying metal grains to iron grains), or a blend of a steel powder and an alloying metal powder optionally together with a partially diffusion-alloyed steel powder. Of various powder metallurgical materials, especially preferred are a blend of an iron-based powder (such as an atomized pure iron powder with an iron content of 90% or more) and an alloying metal powder (such a ferrous alloy powder, a Ni powder, a Cu powder or a Mo powder) and a partially diffusion-alloyed steel powder thereof so as to attain higher compactibility than that attained by a completely alloyed steel powder or the like.

Further, the metal powder has a primary particle size of 75 µm or smaller. When the primary particles of the metal powder are larger than 75 µm in size, the driving force for sintering becomes so weak that that there arise large pores in the sintered body. In the case of using the premix of an iron-based powder and an alloying metal powder (such as a Ni powder a Cu powder or a Mo powder) with a primary particle size greater than 75 µm, alloying metal elements do not diffuse properly in the sintering process. As a result, the sintered body cannot be hardened to a sufficient degree even when heat-treated by e.g. gas carburizing, bright annealing or induction hardening for further improvement in strength, so that the sintered body has a relatively soft and rough ferrite or pearlite structure that can result in fatigue failure. The fatigue strength of the sintered body thus becomes low.

Desirably, the metal powder has been granulated using a binder (such as alumina sol or water glass), or by diffusion joining, so as to agglomerate the primary particles into secondary particles having a particle size of 180 µm or smaller. The granulation of the metal powder increases the apparent particle size and fluidity of the metal powder. As the mechanical properties of the sintered body depends on the primary particle size of the raw material, the fatigue strength of the sintered body does not become lowered as compared with a case where the metal powder has not been granulated. When the secondary particles of the metal powder are larger than 180 µm in size, the packability of the metal powder into a thin area becomes low.

The metal powder can be classified by screening for control of the primary and secondary particle sizes. Namely, the primary particle size of the metal powder can be controlled to 75 µm or smaller by, before the granulation process, passing the metal powder through a screen mesh having a mesh size of 75 µm (200 mesh) as defined by JIS Z8801. Further, the secondary particle size of the metal powder can be controlled to 180 µm or smaller by passing the granulated metal powder through a screen mesh having a mesh size of 180 µm (80 mesh) as defined by JIS Z8801.

The graphite powder is contained in the metal powder mixture in an amount of 0.05 to 1.0% based on the total mass of the metal powder mixture, such that graphite becomes dispersed throughout the sintered body for solid-solution strengthening. When the amount of graphite powder exceeds 1.0%, the green compact becomes low in density. When the amount of graphite powder is less than 0.1%, the graphite powder fails to provide a sufficient solid-solution strengthening effect.

The powder lubricant is contained in the metal powder mixture in an amount of 0.05 to 0.80% based on the total mass of the metal powder mixture, so as to increase the mobility of the solid particles of the metal powder mixture and thereby improve the compactibility of the metal powder mixture. When the amount of powder lubricant is less than 0.05%, the powder lubricant fails to provide sufficient lubricity so that the green compact becomes low in density. In addition, the compact is susceptible to green cracking. When the amount of powder lubricant exceeds 0.80%, the powder lubricant keeps the powder mixture from plastic deformation rather than provides lubricity. The density of the green compact thus becomes so low that the sintered body decreases in density.

The powder lubricant usable in the metal powder mixture is not particularly restricted and can be selected from various lubricating materials to be released in the sintering process. Specific examples of the powder lubricant include metallic soaps such as zinc stearate, lithium stearate and calcium stearate, and waxes such as ethylene-bis-stearoamide. These lubricant compounds can be used alone or in any combination thereof.

The metal powder mixture is compacted while being heated to e.g. 100°C or higher, so as to densify the green compact and thereby reduce the size of pores between the particles and increase contact between the particles. When the temperature of the metal powder mixture in the compacting process is too high, there is a possibility that the powder lubricant melts to deteriorate the fluidity of the powder mixture. The highest temperature of the metal powder mixture in the compacting process is thus preferably limited to 150°C.

If the heated metal powder mixture is compressed into an unheated die, the metal powder mixture becomes cooled. In addition, there occurs heat transfer from the metal powder mixture to the die by the time the compacting process is completed. In view of such circumstances, the die is preferably preheated to a temperature higher than the temperature of the metal powder mixture, e.g. 120°C or higher.

Further, the metal powder mixture is desirably compacted with a die lubricant applied to an inner surface of the die, so as to minimize the amount of powder lubricant contained in the metal powder mixture and thereby increase the density and strength of the sintered body. The die lubricant usable is basically the same as the powder lubricant, such as zinc stearate, lithium stearate and calcium stearate or ethylene-bis-stearamide. In the case of applying the die lubricant by an electrostatic method, the die lubricant needs to be selected in view of its electrostatic property.

The process of applying the die lubricant to the die is not particularly restricted. For example, the die lubricant can be electrostatically adhered to the die by injecting a charged solid powder of die lubricant into the die. The amount of die lubricant applied to the die is desirably 5 to 100 g/m². When the amount of die lubricant is less than 5 g/m², the above-mentioned effects cannot be obtained due to inadequate die lubrication. Moreover, the force to remove the compact from the die becomes large. When the amount of die lubricant exceeds 100 g/cm², the die lubricant remains on a surface of the green compact, thereby resulting in deteriorated appearance.

The green compact is desirably sintered at a temperature of 1180°C or higher in an endothermic gas atmosphere (RX atmosphere), a hydrogen-containing nitrogen atmosphere or an ammonolysis atmosphere, or in a vacuum. In combination with close packing of the metal powder mixture in the compacting process, the sintering of the green compact at such a high temperature effectively promote the diffusion of the particles in the sintering process so as to form stronger bonding between the particles and to densify the sintered body. However, the cost of sintering increases with increase in the sintering temperature. It is thus necessary to select the sintering temperature appropriately for strength/cost tradeoffs.

The sintered body may be given any heat treatment as needed so as to increase in surface hardness and thereby obtain a further improvement in strength. The heat treatment is not particularly restricted and can be a known treatment, such as gas carburizing, bright annealing or induction hardening.

The thus-produced sintered body has a sintered structure derived from the fine metal powder, i.e., a coherent bonded structure formed of sintered metal particles. (The "sintered metal particles" are herein defined as including agglomerates of pluralities of powder particles formed in the sintering process.)

The sintered metal particles have a maximum particle size of 100 µm or smaller. (Herein, the "maximum particle size" refers to the largest diameter of the particles.) When the maximum size of the sintered metal particles is larger than 100 µm, the pore size of the sintered body is too large so that the initial defect of the sintered body that can result in exfoliation abrasion increases in size. The sintered body thus becomes low in strength and abrasion resistance.

Further, the sintered body contains 0.05 to 1.0% of carbon derived from the graphite powder and carbon of the metal powder and dispersed in the sintered structure, based on the total mass of the sintered body. It is noted that a maximum of 0.05% of carbon is burned down in the sintering process.
When the amount of carbon in the sintered body is less than 0.05%, the sintered body cannot attain desired strength and abrasion resistance. When the amount of carbon in the sintered body exceeds 1.0%, the sintered body is so hard as to be susceptible to sintering crack and embrittlement.

It is therefore possible in the present invention to reduce the pore size of the sintered body and to maximize the particle-to-particle contact and particle-to-particle bonding of the sintered body, thereby preventing the pores from being linked together to cause cracking in the sintered body. The produced sintered body advantageously shows excellent fatigue strength and abrasion resistance to be fit for use as a sprocket of an silent chain.

Teeth of the sprocket are susceptible to abrasion as the sprocket teeth receive, from the silent chain, a high surface pressure and a large impactive load accompanied by slippage. The abrasion of the sprocket teeth is classified as "exfoliation abrasion" in which cracking occurs and develops due to the link-up of pores in the sprocket to cause exfoliation in a surface of the sprocket teeth. It becomes however possible to effectively protect the sprocket from such exfoliation abrasion by applying the above sintered body to the sprocket, because the sintered body is small in pore size, large in particle-to-particle contact and high in particle-to-particle bond strength. For cost reduction, the above sintered body may be applied only to the teeth of the sprocket while applying a low-priced material to other portions of the sprocket. For example, the sprocket may be produced by classifying a powder metal into a fine powder having a primary particle size of 75 µm or smaller and a residual powder, and then, using the fine powder for the teeth of the outer peripheral portion of the sprocket while using the residual powder for the inner peripheral portion of the sprocket, thereby reducing the cost of raw materials.

The present invention will be described in more detail by reference to the following examples. However, it should be noted that the following examples are only illustrative and not intended to limit the invention thereto.

### 1. Rotating Bending Fatigue Test

Each test sample was produced by the following procedure.

A partially diffusion-alloyed steel powder (as a fine metal powder) comprised of 4% of Ni, 0.5% of Mo, 1.5% of Cu and the balance being Fe was mixed with a graphite powder and ethylene-bis-stearamide (as a powder lubricant) by the use of a V-blender, thereby providing a metal powder mixture as a raw material. Herein, the partially diffusion-alloyed steel powder had been formed by classifying an atomized pure iron powder by screening, blending the classified iron powder with a powder of Ni, Mo and Cu (having a particle size of 1 to 10 µm), heat-treating the blend at 850°C in such a manner as to adhere alloying metal elements ofNi, Mo and Cu to iron grains by diffusion joining, and then, classifying the resultant granulated powder by screening. The maximum primary and secondary particle sizes of the metal powder and the amounts of graphite powder and powder lubricant added in the metal powder mixture were controlled as indicated in TABLE.

Subsequently, a die was preheated to a given temperature. Then, the metal powder mixture was heated to a given temperature and compacted in the preheated die by the application of a pressure of 686 MPa (7 t/cm²), thereby forming a green compact with a length of 80 mm, a width of 15 mm and a height of 15 mm. Prior to the compacting process, zinc stearate (as a die lubricant) was electrostatically adhered to an inner surface of the die in Examples 2 and 3 and Comparative Examples 2 to 4. The amount of die lubricant applied to the die was 10 g/m². The green compact was sintered at a given temperature for 1 hour in an N₂ atmosphere containing 10 vol% of H₂, thereby providing an iron-based sintered compact. In each example, the heat temperatures of the metal powder mixture and the die in the compacting process and the sintering temperature were controlled as indicated in TABLE.

A test sample having a parallel portion diameter of 8 mm and a straight portion length of 15.4 mm was cut from the sintered compact and then heat-treated under the following conditions.

### (Heat-Treatment Conditions)

Example 1 and Comparative Example 1: subjected to bright annealing, i.e., heated at 900°C for 1 hour, oil-quenched at 60°C, and then, tempered at 180°C for 1 hour.
Examples 2 to 4 and Comparative Examples 3 and 4: subjected to gas carburizing, i.e., heated at 900°C for 2 hours in a carburizing atmosphere with a carbon potential of 0.9%.
The test sample of Comparative Example 2 was given no heat treatment.

The thus-produced test samples of Examples 1 to 4 and
Comparative Examples 1 to 4 were subjected to rotating bending fatigue test according to JIS Z 2274. In the test, the fatigue limit was defined as 10⁷ cycles and evaluated as a rotating bending fatigue strength. The test results are shown in TABLE.

Further, the densities of the green compacts and the heat-treated sintered compacts of Examples 1 to 4 and Comparative Examples 1 to 4 were measured by so-called Archimedes method, in which the volume of a measuring object is calculated by immersing the measuring object in ethanol. The test results are shown in TABLE.

For observation by an optical microscope, the heat-treated sintered compacts of Example 3 and Comparative Examples 3 and 4 were cut in half, and then, the resultant sample pieces were embedded in resinous sample stages and polished. The thus-obtained samples were microscopically examined to observe sintered structures of Example 3 and Comparative Examples 3 and 4 and determine a maximum size of the sintered metal particles of each sintered structure in a observation field of 63 mm x 92 mm. The results are shown in TABLE and FIGS. 3 and 4.

### 2. Abrasion Resistance Test

In each of Examples 1 to 4 and Comparative Examples 1 to 4, a sprocket having 42 involute gear teeth (tooth width: 8.4 mm, over-pin diameter: 84.88 mm, gauge-pin diameter: 3.492 mm) was produced in the same manner as in the production of the above test sample. The produced sintered sprocket was attached to a camshaft of an in-line four-cylinder, 1.8-liter gasoline engine with another sprocket attached to a crankshaft of the engine. The sintered sprocket and the other sprocket were linked by a 5- by 4-row silent chain (pitch: 6.35 mm, effective width: 10.9 mm), and then, the crankshaft was driven by an electric motor under the following conditions to examine an abrasion loss of the teeth of the sprocket of each example. The test results are indicated in FIGS. 1 and 2. In FIGS. 1 and 2, the abrasion loss of the sprockets of Examples 2 to 4 and Comparative Examples 1 to 4 are indicated with respect to the abrasion loss of the sprocket of Example 1 as being represented by 1 (one).

### (Test Conditions)

Tension of Silent Chain: 1500 N (one sided tensioning)
Engine Speed (Crankshaft Rotational Speed): 6000 rpm
Test Time: 100 hours
Lubricant: 5W30SG
Lubricant Temperature: 110°C

In each of Examples 1 to 4, the metal powder mixture was prepared by mixing the metal powder having a primary particle size of 75 µm of smaller and a secondary particle size of 180 µm or smaller with the above-specific amounts of graphite powder and powder lubricant, compacted and then sintered. The sintered metal particles of the resultant sintered body of Example 3 had a maximum particle size of 100 µm or smaller, although the primary particle size of the metal powder of Example 3 was larger than those of Examples 1, 2 and 4. It is estimated that the sintered metal particles of the sintered bodies of Examples 1, 2 and 4 also had a maximum particle size of 100 µm or smaller in consideration of the interrelationship between the primary particle size and the maximum sintered metal particle size. Accordingly, the sintered bodies of Examples 1 to 4 had high fatigue strength and abrasion resistance as indicated in TABLE and FIGS. 1 and 2. The temperature of the metal powder mixture in the compacting process was lower in Example 4 than in Examples 1 to 3, and die lubrication was not performed in Example 4 (not part of the invention). This resulted in lower green density and sintered density. The sintered body of Example 4 however had high fatigue strength and abrasion resistance, benefiting from the effect of using the above-mentioned fine metal powder as a raw material.

On the other hand, the metal powders of Comparative Examples 1 and 2 had a primary particle size larger than 75 µm. On the analogy of Comparative Example 3, it is estimated that the sintered metal particles of the sintered bodies of Comparative Examples 1 and 2 had a maximum size exceeding 100 µm. The sintered bodies of Comparative Examples 1 and 2 were therefore low in fatigue strength and abrasion resistance. The metal powder of Comparative Example 4 also had a primary particle size larger than 75 µm. Further, the amount of powder lubricant added in the metal powder mixture was too much in Comparative Example 4. This resulted in low sintered density and a maximum sintered metal particle size exceeding 100 µm. Thus, the sintered body of Comparative Example 4 was also low in fatigue strength and abrasion resistance. The sintered body of Comparative Example 3 had a maximum sintered metal particle size larger than 100 µm. The fatigue strength of the sintered body of Comparative Example 3 was thus similar to those of the low-density sintered bodies of Comparative Examples 1, 2 and 4, although the sintered body of Comparative Example 3 was relatively high in density. Further, the abrasion resistance of the sintered body of Comparative Example 3 was low.

As described above, the sintered body can be produced by preparing the metal powder mixture from the fine metal powder, the graphite powder and the powder lubricant, warm-compacting the metal powder mixture optionally with die lubrication, and then, sintering the compacted powder mixture at a relatively high temperature in the present invention. If necessary, the metal powder may be granulated to a desired particle size. This makes it possible to provide the sintered body with a very small pore size, maximized particle-to-particle contact, strong particle-to particle bonding and high sintered density, thereby effectively preventing the occurrence and development of cracking in the sintered body effectively. In addition, there is no need to repeat the compaction and sintering processes for increased green density and sintered density. The sintered body is therefore produced at relatively low cost while attaining significantly improved fatigue strength and abrasion resistance to be suitable for use in a sprocket of a silent chain or a high-strength part of an internal combustion engine.

The entire contents of Japanese Patent Application No. 2003-009483 (filed on January 17,2003).

Although the present invention has been described with reference to specific embodiments of the invention, the invention is not limited to the above-described embodiments. Various modification and variation of the embodiments described above will occur to those skilled in the art in light of the above teaching. The scope of the invention is defined with reference to the following claims.

## Claims

1. A production method of a sintered body forming at least teeth of a sprocket of a silent chain, comprising:
sintered metal particles forming a sintered structure
and having a maximum particle size of 100 µm or smaller; and carbon being dispersed in the sintered structure in an amount of 0.05 to 1.0% by mass based on a total mass of the sintered body, the method comprising:
preparing a metal powder mixture, the metal powder mixture including a fine metal powder having a particle size of 75 µm or smaller, a graphite powder in an amount of 0.1 to 1.0% by mass and a powder lubricant in an amount of 0.05 to 0.80% by mass based on a total mass of the metal powder mixture;
compacting the metal powder mixture to provide a green compact; and
sintering the green compact, wherein the metal powder mixture is compacted while being heated to a temperature of 100°C or higher.

2. A production method according to claim 1,
wherein the metal powder is a blend of an iron-based powder and an alloying metal powder.

3. A production method according to any one of Claims 1 to 2,
wherein said preparing includes granulating the metal powder to form primary particles having a particle size of 75 µm or smaller into secondary particles having a particle size of 180 µm or smaller.

4. A production method according to any of Claims 1 to 3,
wherein said compacting includes preheating a die to a temperature of 120°C or higher, and then, compressing the metal powder mixture into the preheated die.

5. A production method according to any one of Claims 1 to 4,
wherein said compacting includes applying a die lubricant to a die, and then, compressing the metal powder mixture into the die.

6. A production method according to any one of Claims 1 to 5,
wherein the green compact is sintered at a temperature of 1180°C or higher.

7. A production method according to any one of Claims 1 to 6, further comprising heat-treating the sintered compact.

## Patentansprüche

1. Verfahren zur Herstellung eines gesinterten Körpers, der zumindest Zähne eines Kettenrads einer geräuschlosen Kette bildet, umfassend:
gesinterte Metallpartikel, die eine gesinterte Struktur bilden und eine maximale Partikelgröße von 100 µm oder kleiner aufweisen;
und Kohlenstoff, der in der gesinterten Struktur in einer Menge von 0,05 bis 1,0 Gew.% auf der Grundlage einer Gesamtmasse des gesinterten Körpers verteilt ist, wobei das Verfahren umfasst:
Herstellen einer Metallpulvermischung, wobei die Metallpulvermischung ein Feinmetallpulver mit einer
Partikelgröße von 75 µm oder kleiner, ein Graphitpulver in einer Menge von 0,1 bis 1,0 Gew.% und ein Pulverschmiermittel in einer Menge von 0,05 bis 0,80 Gew.% auf der Grundlage einer Gesamtmasse der Metallpulvermischung umfasst;
Verdichten der Metallpulvermischung, um einen Grünling zu bilden; und
Sintern des Grünlings, wobei die Metallpulvermischung verdichtet wird, während sie auf eine Temperatur von 100 °C oder höher erwärmt wird.

2. Herstellungsverfahren nach Anspruch 1, wobei das Metallpulver eine Mischung aus einem eisenbasierten Pulver und einem legierten Metallpulver ist.

3. Herstellungsverfahren nach einem der Ansprüche 1 bis 2, wobei die Herstellung ein Granulieren des Metallpulvers umfasst, um primäre Partikel mit einer Partikelgröße von 75 µm oder kleiner in sekundäre Partikel mit einer Partikelgröße von 180 µm oder kleiner umzuformen.

4. Herstellungsverfahren nach einem der Ansprüche 1 bis 3, wobei das Verdichten ein Vorheizen einer Gussform auf eine Temperatur von 120 °C oder höher und dann ein Komprimieren der Metallpulvermischung in der vorgeheizten Gussform umfasst.

5. Herstellungsverfahren nach einem der Ansprüche 1 bis 4, wobei das Verdichten ein Aufbringen eines Gussform-Schmiermittels auf eine Gussform und dann ein Komprimieren der Metallpulvermischung in der Gussform umfasst.

6. Herstellungsverfahren nach einem der Ansprüche 1 bis 5, wobei der Grünling bei einer Temperatur von 1180 °C oder höher gesintert wird.

7. Herstellungsverfahren nach einem der Ansprüche 1 bis 6, ferner umfassend eine Wärmebehandlung des gesinterten Presskörpers.

## Revendications

1. Procédé de production d'un corps fritté formant au moins des dents d'un pignon d'une chaîne silencieuse, comprenant : des particules métalliques frittées formant une structure frittée et ayant une taille particulaire maximum de 100 µm ou moins ; et du carbone qui est dispersé dans la structure frittée selon une quantité de 0,05 à 1,0 % en masse en fonction d'une masse totale du corps fritté,
le procédé comprenant les étapes consistant à:
préparer un mélange de poudre de métal, le mélange de poudre de métal comprenant une poudre métallique fine ayant une taille particulaire de 75 µm ou moins, une poudre de graphite selon une quantité de 0,1 à 1,0 % en masse et un lubrifiant en poudre selon une quantité de 0,05 à 0,80 % en masse en fonction d'une masse totale du mélange de poudre de métal ;
compacter le mélange de poudre de métal pour donner un comprimé non fritté ; et
fritter le comprimé non fritté, dans lequel le mélange de poudre de métal est compacté tout en étant chauffé à une température de 100 °C ou plus.

2. Procédé de production selon la revendication 1, dans lequel la poudre métallique est un mélange d'une poudre à base de fer et d'une poudre métallique d'alliage.

3. Procédé de production selon l'une quelconque des revendications 1 à 2, dans lequel ladite étape de préparation comprend l'étape consistant à présenter sous forme de granulés la poudre métallique pour former des particules principales ayant une taille particulaire de 75 µm ou moins en particules secondaires ayant une taille particulaire de 180 µm ou moins.

4. Procédé de production selon l'une quelconque des revendications 1 à 3, dans lequel ladite étape de compactage comprend l'étape consistant à préchauffer un moule à une température de 120 °C ou plus, et ensuite comprimer le mélange de poudre métallique dans le moule préchauffé.

5. Procédé de production selon l'une quelconque des revendications 1 à 4, dans lequel ladite étape de compactage comprend l'étape consistant à appliquer un lubrifiant pour moule sur un moule, et ensuite à comprimer le mélange de poudre de métal dans le moule.

6. Procédé de production selon l'une quelconque des revendications 1 à 5, dans lequel le comprimé non fritté est fritté à une température de 1180 °C ou plus.

7. Procédé de production selon l'une quelconque des revendications 1 à 6, comprenant en outre l'étape consistant à faire subir un traitement thermique au comprimé fritté.
